

# UNITED STATES PATENT OFFICE.

EDWARD F. KENNEY, OF WESTMONT BOROUGH, PENNSYLVANIA.

## TREATING RAILS.

1,205,998.

Specification of Letters Patent.

Patented Nov. 28, 1916.

No Drawing.

Application filed March 20, 1916. Serial No. 85,479.

To all whom it may concern:

Be it known that I, EDWARD F. KENNEY, a citizen of the United States, residing in the borough of Westmont, in the county of Cambria and State of Pennsylvania, (whose post-office address is Johnstown, Pennsylvania,) have invented certain new and useful Improvements in Treating Rails; and I do hereby declare the following to be a full, clear, and exact description of the invention, such as will enable others skilled in the art to which it appertains to make and use the same.

My invention relates to treating steel rails and similar articles after they have been rolled or otherwise formed, for the purpose of making them stronger, tougher and better adapted to withstand the shocks, impacts and wear to which they are subjected when in use. In order to accomplish this in a simple, economical and practical way and one which will be commercially available, I prefer to quench the rails in water, oil or other cooling medium after they have been rolled or otherwise formed and while they are still at the proper heat for this purpose, in order to avoid the necessity and expense of reheating them before quenching. In certain cases, however, I may permit the rails to cool to atmospheric, or similar temperatures, after they have been rolled and then reheat them to the proper temperature for quenching, as I can obtain thereby, equivalent results, but at the expense of a slight additional cost and loss of time.

In order that the rails or other material shall not be badly warped by reason of the cooling and the shrinking of the thinner portions, or those with a greater surface as compared with their volume before the shrinkage of the other and more massive portions, I prefer to deliver them into the cooling bath when they are in a vertical position, or a position slightly inclined from the vertical, in which case the only warping that will be produced is that due to the difference in cooling of the thinner and thicker portions. If, on the other hand, the rail or other material is supported horizontally or approximately so on supports of any kind, it will warp and bend, due to its weight on these supports in addition to the warping due to unequal shrinkage of its different portions, and this will make it impossible or impracticable to straighten and if

attempted will set up undue stresses. In addition to this, I have found that it is not necessary to cool or quench the rail or other material to atmospheric temperature or to that of the cooling medium if at or near atmospheric temperature; but that by cooling it to a lesser extent, I prevent undue shrinkage stresses and cracks. I have also found that rails and other materials which have been quenched and annealed and allowed to cool to approximately atmospheric temperature or that of the cooling medium at or near atmospheric temperature are too hard to straighten without danger of damage, which in their further use would be very disastrous.

In order to obviate setting up of undue stresses after the rails have been quenched, I prefer to straighten them when at a considerable temperature and one at which they are sufficiently plastic to be straightened either by a straightening press or a set of rolls; but this temperature is one which will not affect the amorphous structure produced by the quenching.

Although my invention may be carried out through various ranges of temperatures, I prefer to proceed about as follows, and in order to simplify the language I will refer to temperature on the Fahrenheit scale and to rails alone, although other steel material may be similarly treated, as will be readily understood: I first roll the rails in a rolling mill from a white heat and finish them in the mill at temperatures varying from 1400 degrees to 2000 degrees. After the rail has issued from the mill and a very short time elapsed, it is turned upward preferably while resting on supports distributed throughout its length into a vertical or inclined position while it is at a temperature from about 1350 degrees to 1900 degrees, and it is then lowered and cooled in a bath of cold, warm or hot quenching material, either water, oil or other medium as may be desired. This at once provides an amorphous or very fine structure in the steel and one which puts the material in condition to withstand shocks, impacts and wear of use. This quenching is accomplished rapidly, and the material is withdrawn from the bath before its temperature falls below about 400 degrees. I may, however, as previously stated, allow the rails to cool after rolling and then reheat them prior to quenching, instead of

quenching at their finishing or residual heat. In this method of cooling the structure is held and maintained amorphous or of fine grain, while avoiding cooling down 5 to ordinary atmospheric temperatures and the steel material is more plastic, besides which this method avoids undue temperature stresses that would otherwise crack, or tend toward cracking or undue straining the 10 material. After this is done, I reheat the rails to a temperature above one of the critical temperatures; namely 800 degrees to 950 degrees, which is above what is known as the "blue heat," and one which makes 15 the material very plastic and easy to bend or straighten. This temperature also anneals the material and removes temperature stresses without materially changing the fine or amorphous structure thereof. I then 20 immediately straighten the rail in rolls or a gag press when its temperature is approximately from 600 degrees to 950 degrees. At these temperatures the material is much more plastic and its elastic limit 25 much less than if at atmospheric temperature, and will thus permit straightening without causing undue stresses or strains.

The critical temperature or recalescent point for steel rails is about 1250 degrees, 30 and I take pains not to exceed this in reheating the rails prior to the proposed annealing before straightening them. The results of actual tests of rails treated in this way show that the elastic limit is very much increased, 35 the ultimate strength is considerably increased, the elongation is about the same, the reduction of area is very largely increased, hardness and consequent wearing qualities are increased very much, the bending 40 strength and capacity is almost doubled, the resistance to impact is almost doubled, and the resistance to the drop test is considerably increased, together with an increase in the ductility and stiffness. In straightening 45 the rails in this manner at the temperature stated, I take pains to give them a slight curvature so that when they are cold they will draw substantially straight.

Although I have shown and described my 50 improvements in considerable detail, I do

not wish to be limited to the exact and specific details shown and described, but may use such substitutions, modifications or equivalents thereof as are embraced within the scope of my invention, or as pointed out in the claims.

Having thus described my invention, what I claim and desire to secure by Letters Patent is:—

1. The steps in the method of treating 60 rails, which consists in quenching them in a vertical or slightly inclined position and thereby cooling them to a temperature not less than 400 degrees.

2. The steps in the process of treating 65 rails comprising quenching them at their finishing temperature to a temperature not less than 400 degrees, then heating them to a temperature above 800 degrees, but not to their recalescent temperature, then straightening them while above a temperature of 600 degrees.

3. The process of treating rails, which consists in finishing them at temperatures from 1400 degrees to 2000 degrees, then 75 quenching them to a temperature not less than 400 degrees, then reheating them to temperatures above 800 degrees, but not more than their recalescent temperature, then straightening them before they are at a temperature of less than 600 degrees.

4. The steps in the method of treating rails, which consists in heating them to temperatures from 1400 degrees to 2000 degrees, then quenching them in a vertical or 85 slightly inclined position and thereby cooling them to a temperature not less than about 400 degrees.

5. The process of treating rails, which consists in heating them to temperatures 90 from 1400 degrees to 2000 degrees, then quenching them to a temperature not less than 400 degrees, then reheating them to temperatures above 800 degrees, but not more than their recalescent temperature, 95 then straightening them before they are at a temperature of less than 600 degrees.

In testimony whereof I hereto affix my signature.

EDWARD F. KENNEY.